

Jan. 7, 1936.

C. E. SOSSON  
IGNITION COMPOSITION

2,027,208

Filed Nov. 19, 1934



*Fig. 1*

*Fig. 2*

*Fig. 3*

Charles E. Sosson

BY

*Irvin Sosson*

INVENTOR.

ATTORNEY.

## UNITED STATES PATENT OFFICE

2,027,208

## IGNITION COMPOSITION

Charles Edwin Sosson, Ardrossan, Scotland, assignor to Imperial Chemical Industries Limited, a corporation of Great Britain

Application November 19, 1934, Serial No. 753,778  
In Great Britain November 21, 1933

10 Claims.

(Cl. 52—4)

This invention relates to ignition compositions and more particularly to a new and improved ignition mixture which gives rise to little or no gas on combustion.

5 Ignition mixtures which have heretofore been widely employed in the art have been unsatisfactory for many purposes because of the large volume of gases generated during combustion. These gases were particularly objectionable in 10 delay detonators, since the hot gases were known to produce premature detonations and at times to cause the undesirable burning of the dynamite. Various attempts have been made, therefore, to develop gasless ignition mixtures or compositions 15 giving off relatively small volumes of gas which would be satisfactory for use in electric blasting devices. The present invention proposes a more satisfactory solution to the problem.

The object of my invention is an improved ignition mixture. A further object is an ignition mixture which produces little or no gas on combustion and which is particularly advantageous for use in delay detonators. Other objects will appear as the invention is hereinafter disclosed.

25 I have found that these objects may be accomplished by the following invention, which consists essentially in the employment of an ignition composition comprising zirconium and an easily ignitable lead salt of a nitrophenol.

30 According to my invention, the material directly ignitable by the passage of the electric current consists of a quantity of finely divided zirconium together with basic lead 2-mono-nitro resorcinate, basic lead picrate or other easily ignitable lead salt of a nitrophenol having a suitably low firing current, preferably below 0.5 amps. when the current is applied for a period of 50 milliseconds. While previous low tension ignition compositions containing basic lead 2-mono-nitro 35 resorcinate have shown considerable advantage, those made in accordance with the present invention provide an even greater degree of certainty in ignition.

The zirconium is advantageously employed in 40 a fine state of division, e. g. having a particle size not greater than 0.005 mm., and preferably substantially less.

The proportion of zirconium to basic lead 2-mono-nitro resorcinate or other lead salt of a 45 nitrophenol may vary within wide limits. I prefer, however, that the ratio should be high, since the compositions containing the higher proportions of zirconium yield a more powerful flash. Beneficial results are obtained with compositions 50 in which the ratio of zirconium to lead salt is

50/50 but preferably the ratio lies between 35/65 and 95/5. It is not, however, advisable to exceed the last mentioned proportion since the firing current then becomes unduly high. In general, the best results are obtained as regards firing and freedom from gas when the proportion of zirconium to lead salt is at least 70 to 30. Various types of electric ignition devices may be employed in carrying out my invention, such as for example the well known concave plug, the bridge plug 10 type, or a form of match head. When necessary the mixture of zirconium and lead salt may be made into a coherent form with the aid of a small quantity of a suitable cementing material such as nitrocellulose.

15 The fact that the compositions comprising finely divided zirconium and lead salts of the kind described produce little or no gas on combustion, together with the fact that they produce a powerful flash, renders the invention especially advantageous for use in delay action detonators of the ventless type. Since the compositions employed in the delay elements of such detonators are usually less easily ignited than ordinary delay fuse compositions, I prefer to use fairly high 20 proportions of zirconium to lead salt, for example 70 to 30 or higher. In the construction of the firing devices intended for such uses, the diameter of the bridge wires may be somewhat reduced in order to prevent the increase in the firing current 25 which would otherwise be necessary when the proportion of zirconium to lead salt rose above 70 to 30.

30 Moreover, the presence of other materials yielding gases should be avoided when the here- 35 described invention is used in ventless delays. In all other types of detonators, various materials customarily employed to give a better flash may be used, if desired, but this is quite unnecessary according to the present invention. 40

In order to illustrate the use of my invention more fully, I may cite the following examples which are diagrammatically represented in the attached drawing. Figure 1 represents a vertical section of an electric blasting cap using the 45 bridge plug type of ignition, Figure 2 represents a delay electric blasting cap having a match head igniter, while Figure 3 represents a similar section of a delay detonator having a concave plug type igniter.

50 In Figure 1, the shell A contains a base charge B and a primary charge C covered with a loose ignition mixture D, comprising 70 parts zirconium and 30 parts basic lead 2-mono-nitro resorcinate. The bridge wire E is connected to the leading 55

wires F held in bridge plug G and embedded in the ignition mixture. The shell is sealed by a waterproofing composition H and a sulfur seal I.

In Figure 2, representing a delay cap utilizing 5 a match head igniter, the shell A of the detonator contains a base charge B and a primary charge C, covered with a loose ignition mixture D comprising 70 parts zirconium and 30 parts basic lead 2-mono-nitro resorcinate. Above this mixture 10 is positioned a delay element E containing any suitable gasless delay ignition mixture F. The upper end of the delay element is separated by the space G from the match head composition H, which is prepared by dipping the bridge wire 15 connecting the lead wires I into a suspension of a mixture of 70 parts zirconium powder and 30 parts basic lead 2-mono-nitro resorcinate in a sufficient amount of a 5% solution of nitrocellulose in commercial amyl acetate to make a creamy mixture. The bead formed on the bridge wire is then dried, dipped into a waterproofing solution of collodion, and dried again. The leading wires I pass through the plug J, held in the detonator by the crimp K. The open end of the detonators is 20 then closed with the sealing compound L.

In Figure 3, representing a delay detonator having a concave plug igniter, the shell A contains a base charge B and a primary charge C, covered by a loose ignition mixture D, comprising 70 parts zirconium and 30 parts basic lead 2-mono-nitro resorcinate. Above this mixture is a delay element E containing any suitable gasless delay ignition mixture F. The upper end of the delay element is separated by the space G from a plug H having a concave face and a bridge wire I between two leading wires J. The concave plug is covered with a paste comprising 70 parts zirconium, 30 parts basic lead 2-mono-nitro resorcinate and sufficient 5% amyl acetate solution of 30 nitro-cellulose to give the mixture the desired consistency. After this has dried, the concave mixture is waterproofed, dried again, and assembled in the delay detonator in the usual manner. It is held in place by a waterproofing composition K and a sulfur seal L.

Having now described and illustrated my invention in detail, it is apparent that many variations can be made without departing from the

spirit of the invention. The above examples are illustrative only and are not intended to limit the invention to these particular embodiments. I intend, therefore, to be limited only to the extent indicated by the following patent claims. 5

I claim:

1. An ignition composition comprising zirconium and an easily ignitable lead salt of a nitrophenol.
2. An ignition composition comprising 50 to 10 95% zirconium and 50 to 5% of an easily ignitable lead salt of a nitrophenol.
3. An ignition composition comprising 50 to 95% zirconium and 50 to 5% basic lead 2-mono-nitro resorcinate.
4. An ignition composition comprising approximately 70% zirconium and approximately 30% basic lead 2-mono-nitro resorcinate.
5. An ignition composition as the firing charge in an electric blasting cap, said composition possessing low firing current requirements and comprising 50 to 95% zirconium and 50 to 5% of an easily ignitable lead salt of a nitrophenol.
6. An ignition composition as the firing charge in a delay detonator, said composition comprising 50 to 95% zirconium and 50 to 5% of an easily ignitable lead salt of a nitrophenol.
7. An ignition composition as the firing charge in an electric delay detonator, said mixture comprising 50 to 95% zirconium and 50 to 5% basic lead 2-mono-nitro resorcinate.
8. An ignition composition as the firing charge in an electric delay detonator, said mixture comprising approximately 70% zirconium and approximately 30% basic lead 2-mono-nitro resorcinate.
9. A cemented ignition composition as the firing charge in a ventless electric delay detonator, said mixture comprising not less than 70% zirconium and not more than 30% basic lead 2-mono-nitro resorcinate.
10. A cemented ignition composition as firing charge in a ventless electric delay detonator comprising an ignitable mixture together with a small quantity of a cement, the said mixture consisting of not less than 70% zirconium and not more than 30% basic lead 2-mono-nitro resorcinate.

CHARLES EDWIN SOSSON.